

# United States Patent [19]

Volin

[11] 3,877,930

[45] Apr. 15, 1975

[54] **ORGANIC INTERDISPERSION COLD BONDING CONTROL AGENTS FOR USE IN MECHANICAL ALLOYING**

3,740,210 6/1973 Bomford et al. .... 75/5 AC

[75] Inventor: Timothy Earl Volin, Tuxedo, N.Y.

## OTHER PUBLICATIONS

[73] Assignee: The International Nickel Company, Inc., New York, N.Y.

"The Role of Additives in Milling," A Treatise on the Internal Mechanisms of Ball, Tube and Rod Mills, H.E. Rose and R.M.E. Sullivan, 1958, pp. 236-251.

[22] Filed: Jan. 29, 1973

Primary Examiner—L. Dewayne Rutledge  
Assistant Examiner—Arthur J. Steiner  
Attorney, Agent, or Firm—Ewan C. MacQueen;  
Raymond J. Kenny

[21] Appl. No.: 327,321

[52] U.S. Cl. .... 75/0.5 R; 75/5 AB; 75/5 BA;  
75/211; 75/171

[51] Int. Cl. .... B22f 9/00

[58] Field of Search..... 75/5 R, 214, 211, 171;  
241/15; 264/111

## [56] References Cited

### UNITED STATES PATENTS

|           |         |                     |        |
|-----------|---------|---------------------|--------|
| 2,995,780 | 8/1961  | West et al.....     | 18/48  |
| 3,301,494 | 1/1967  | Lonquist et al..... | 241/22 |
| 3,479,180 | 11/1969 | Lambert et al. .... | 75/206 |

[57]

## ABSTRACT

The invention involves mechanical alloying of powder wherein the formation of composite powder particles characteristic of the mechanical alloying process is facilitated through the use of special organic interdispersion cold bonding agents, e.g., stearic acid. The invention is particularly applicable to the production of non-dispersion hardening superalloys.

2 Claims, No Drawings

# ORGANIC INTERDISPERSION COLD BONDING CONTROL AGENTS FOR USE IN MECHANICAL ALLOYING

The present invention relates to powder metallurgy, and is particularly directed to the "mechanical alloying" of powder.

As is known, the recently introduced concept of "mechanical alloying," described in U.S. Pat. No. 3,591,362 (incorporated herein by reference), involves a dry, intensive milling of powders in high energy machines, such as the Szegvari attritor. During this unique process, initial constituent powders are repeatedly fragmented and cold bonded by the continuous impacting action of attriting elements, usually metal balls, for a period such that composite product powder particles of substantial saturation hardness are formed, the composition of which correspond to the percentages of the respective constituents in the original charge. The constituent powders become most intimately interdispersed at close interparticle spacings, the composite particles being exceptionally dense and homogeneous, and characterized by cohesive internal structures.

For the most part "mechanical alloying" (often herein "MA") has been conducted in the presence of an atmosphere comprised of an oxygen-nitrogen mixture. However, such an environment can serve to introduce various problems, particularly in respect of non-dispersion strengthened alloys of the superalloy type. For example, oxygen is retained in the composite product particles formed. As a consequence and depending upon the alloy composition to be produced, this can subvert certain metallurgical properties, tensile and creep ductility of nickel-base superalloys being illustrative. Moreover, if present to the excess, comminution of the powders dominates to such an extent as to virtually preclude the critically necessary cold bonding.

On the other hand, in the absence of such atmospheres the powders either adhere irreversibly to the attriting elements and interior attritor surfaces (with subsequent buildup) or, depending upon the composition of the attriting elements and powder charge, may irreversibly cold bond to form undesirably large particles. In the former case the layer bonded to the balls, and in the latter case the large particles, are too thick to be satisfactorily deformed by the energy available in subsequent collision events. Processing therefore effectively ceases. Indeed, a point may be reached where there is such an overload on the attritor as to bring about a self-induced shut-down. This, quite naturally, leads to considerable loss occasioned by down-time. In any case, powder recovery is extremely poor.

It is evident from the foregoing that an indispensably necessary mechanical alloying "control balance" must be achieved, this "control balance" being defined as one in which the intimate interdispersion of constituent powders continues by means of the establishment of steady state processing (fragmentation and cold bonding reaching a virtual equilibrium), but (i) without incurring serious impairment of the metallurgical properties of the alloy to be produced due, for example, to excessive oxygen retention in non-dispersion strengthened alloys, (ii) without the formation of appreciable quantities of detrimentally large composite product particles, and (iii) without the deleterious adherence of powders to the attriting (milling) elements or other attritor surfaces.

It has now been discovered that the above drawbacks can be considerably minimized, if not virtually eliminated, that the desired "control balance" can be attained, through incorporating an effective percentage of at least one interdispersion, cold-bonding agent (ICBCA), as herein detailed.

Generally speaking, it has been found that an organic agent, including organometallic compounds, capable of reacting with or of being adsorbed on a plurality of the powder (particle) surfaces of an initial powder charge and which is capable of residing thereof in reacted or adsorbed form during at least a significant part of the "mechanically alloying" process, is effective in achieving the aforescribed "control balance". (Such materials include organic compounds which decompose such as to form a constituent capable of reacting with or of being adsorbed on the powder surfaces.) Only a small quantity of the organic ICBCA is required, though this is dependent upon the given conditions used in producing the desired mechanically alloyed composite product powder particles as is further described herein.

In accordance herewith, ICBCAs such as the following are contemplated: saturated hydrocarbons such as 25 methane, ethane, propane and hexane; unsaturated hydrocarbons such as ethylene, allene, hexene and acetylene; alcohols, including methanol, ethanol, and ethylene glycol; aldehydes, e.g., formaldehyde, trioxane, acetylaldehyde, and benzaldehyde; ethers, for example, methyl or vinyl ether; ketones, such as acetone; polymers of the foregoing; organohalogen compounds, including the carbon tetrahalides such as  $CF_4$ , and polymers thereof such as polytetrafluoroethylene; organometallic compounds, for example, nickel or cobalt 30 stearate, triethylaluminum, dicyclopentadiene-nickel, nickel tetracarbonyl; fats and fatty acids such as stearic acid, stearin, and the formic, oleic, and oxalic acids; etc. (This listing is not intended to be exhaustive.) It is considered that such materials by virtue of their reacting with or being adsorbed on the surfaces of the powder particles are occluded during collisional events between powder particles and this inhibits metal-to-metal bonding. This largely contributes to the desired "control balance."

The amount of an ICBCA employed will be largely influenced, *inter alia*, by the alloy composition to be produced, milling time, machine design and speed, ball-to-powder ratio, and the nature of the attriting elements, particularly the latter. Hardened steels, stainless steels, tungsten carbide, nickel and other metals as well as cermets may be used as the attriting media; however, considerably less ICBCA will usually be necessary in conjunction with the harder attriting elements such as 52,100 steel as opposed to, say, nickel. The longer milling periods may require a slightly higher percentage of ICBCA than otherwise. Generally, not more than 2 or 3 percent of an effective ICBCA component need be employed, a range of 0.05 or 0.1 to 0.5 percent and up to 2 percent being deemed satisfactory. Excessive amounts can be detrimental. In terms of a hydrocarbon such as, for example, acetylene, about 0.025 to 2 percent carbon as hydrocarbon can be used, with 0.05 to 0.5 percent being considered advantageous.

Due to the high energy milling of mechanical alloying, a part of the attriting composition may wear during processing and become a part of the composite product particles. This can be beneficial but if undesirable, re-

course should be had to a more appropriate attriting composition.

It is perhaps worthy of mention that not all of the ICBCA can be removed and this does focus attention on a major difference between the subject invention and conventional ball milling in which surfactants, lubricants and other grinding aids are used for various purposes, mainly for powder comminution. Generally, the latter are virtually completely removed from the powder by expedients such as leaching or burning off. In contrast, due to the necessary intimate interdispersion of constituent powders which occurs by reason of "mechanical alloying," removal techniques affecting only the composite particle powder surfaces are incapable of extricating all the ICBCA since an amount of it is occluded in interdispersion fashion.

The following illustrative data are given:

#### EXAMPLE

Composite product powder particles of the alloy known as IN-792 were produced using various ICBCAs and either nickel or steel attriting elements. Powder blends were used, each being comprised of carbonyl nickel powder (99.1 percent nickel approximately 4 microns in size), 0.15 percent Asbury flake graphite to raise the carbon content to nominal, and a low oxygen omnibus master alloy (-100 mesh of 30 percent Ni, Cr, Mo, Co, Al, Ti, W, Ta, B, Zr and C) prepared by vacuum induction melting and grinding in cold nitrogen. Each run consisted of 5 grams of the blended powder plus the particular ICBCA used as given in Table I.

A Spex mill was employed in each case, the respective runs being conducted for 30 minutes under an argon atmosphere (atmosphere was acetylene plus argon in Run No. 6). The Spex mill jar was cooled prior to opening, emptied and the balls replaced in the jar and processed for an additional 30 seconds in air to remove any loosely adherent powder. The total amount of drained powder was weighed to ascertain the percentage of powder recovered. An oxygen analysis was also made, and retained ICBCA was determined for Runs. Nos. 4 and 6. Nos. 1 and 2 are included for purposes of comparison.

TABLE I

| Run | ICBCA              | Attriting Element | Powder Recovery (%) | Oxygen Analysis (%) | ICBCA Retained |
|-----|--------------------|-------------------|---------------------|---------------------|----------------|
| 1   | None               | Nickel (100 gm)   | 32                  | 0.30                | —              |
| 2   | None               | Steel (100 gm)    | 57                  | 0.17                | —              |
| 3   | Stearic Acid, 1%   | Nickel (100 gm)   | 81                  | 0.46                | —              |
| 4   | Stearic Acid, 0.1% | Steel (100 gm)    | 81                  | 0.22                | 0.32% C        |
| 5   | PTFE 0.2%          | Nickel (100 gm)   | 65                  | 0.31                | —              |
| 6   | Acetylene*         | Steel (100 gm)    | 78                  | 0.21                | 0.29% C        |

\*atmosphere estimated to be about 10% Acetylene

The low recovery of Run. No. 1 reflects the detrimental adherence of the IN-792 powder to the milling elements and to the interior surfaces of the mill. This was reduced somewhat by using the harder steel impacting elements in Run No. 2. Runs 3 and 4 further illustrate the marked effect of the nature of the attriting elements, only one-tenth of the stearic acid ICBCA being required with steel balls to give the same recovery attained using the softer nickel pellets. It is consid-

ered that the recovery for the polytetrafluoroethylene (PTFE) of Run No. 5 would be improved using steel balls as the attriting elements.

The present invention is particularly applicable to the production of non-dispersion hardening superalloys including those containing up to 65 percent, e.g., from 2 percent up to 25 or 35 percent, chromium; up to 30 percent, e.g., 5 to 25 percent, cobalt; up to 10 percent, e.g., 1 to 9 percent, aluminum, and up to 8 percent, e.g., 1 to 7 percent, titanium, including those alloys containing 4 or 5 percent or more of aluminum plus titanium; up to 30 percent, e.g., 1 to 8 percent, molybdenum; up to 25 percent, e.g., 2 to 20 percent, tungsten; up to 10 percent columbium, up to 10 percent tantalum, up to 7 percent zirconium, up to 0.5 percent boron, up to 5 percent hafnium, up to 2 percent vanadium, up to 6 percent copper, up to 5 percent manganese, up to 70 percent iron, up to 4 percent silicon, and the balance essentially nickel. Cobalt-base alloys of similar composition can be treated. Among the specific superalloys might be listed IN-738, Rene alloys 41 and 95, Alloys 500, 700, 713 and 718, Waspaloy, Astroloy, Mar-M alloys 200 and 246, A-286, B-1900, etc. However, such superalloys and other contemplated alloys can also contain up to, say, 10 percent by volume of a refractory dispersoid material including the oxides, carbides, nitrides and borides. Such refractory dispersoids can be of various elements including yttrium, lanthanum, thorium, zirconium, hafnium, titanium, silicon, aluminum, cerium, uranium, magnesium, calcium, beryllium and the like. As a practical matter, only a very small amount of such dispersoids need be employed, e.g., up to 2 percent by volume. Other base alloys such as titanium and copper can be processed as well as refractory alloys such as SU-16, TZM, Zircaloy, etc.

Finally, it will be understood that modifications and variations of the invention may be resorted to without departing from the spirit and scope thereof as those skilled in the art will readily understand. Such are considered to be within the purview and scope of the invention and appended claims.

I claim:

1. In the process of producing mechanically alloyed

superalloy composite product powder particles consisting of up to 65 percent chromium, up to 10 percent aluminum, up to 8 percent titanium, up to 30 percent molybdenum, up to 25 percent tungsten, up to 10 percent columbium, up to 10 percent tantalum, up to 7 percent zirconium, up to 0.5 percent boron, up to 5 percent hafnium, up to 2 percent vanadium, up to 6 percent copper, up to 5 percent manganese, up to 70 percent iron, and the balance essentially nickel and/or

cobalt, the improvement which comprises conducting the mechanical alloying operation in the presence of an interdispersion cold bonding agent (ICBCA) selected from the group consisting of methane, ethane, propane and hexane, the ICBCA being in contact with the powder particles to be mechanically alloyed and being present in an amount effective to provide the necessary control balance during the course of the operation with the upper limit being not greater than 3 percent by weight of the powder charge, the control balance being such that an intimate interdispersion of constituent

powders is achieved without incurring serious impairment of the mechanical properties of the composition to be produced and without either the formation of an appreciable amount of detrimentally large composite particles or the deleterious adherence of powders to the milling elements or mill interior surfaces.

5 2. A process as set forth in claim 1 in which the ICBCA is methane present in an amount from 0.1 to 10 0.5 percent by weight of the powder charge.

\* \* \* \* \*

15

20

25

30

35

40

45

50

55

60

65